

May 31, 1938.

E. D. VIERS ET AL

2,119,304

ELECTROPLATING

Filed Aug. 1, 1935

2 Sheets-Sheet 1

a



FIG.1

b



FIG.2

c



FIG.3

d



FIG.4

INVENTOR

EUGENE D. VIERS  
and BERNARD C. CASE

BY

Bates, Goluck, & Teare  
ATTORNEYS

May 31, 1938.

E. D. VIERS ET AL

2,119,304

ELECTROPLATING

Filed Aug. 1, 1935

2 Sheets-Sheet 2



FIG. 5 (OLD)



FIG. 6

INVENTOR.

EUGENE D. VIERS  
BY and BERNARD C. CASE  
Bates, Golnick, & Teare  
ATTORNEYS

## UNITED STATES PATENT OFFICE

2,119,304

## ELECTROPLATING

Eugene D. Viers and Bernard C. Case, Cleveland,  
Ohio, assignors to Eaton Detroit Metal Com-  
pany, Cleveland, Ohio, a corporation of Ohio

Application August 1, 1935, Serial No. 34,209

18 Claims. (Cl. 204—14)

This invention relates to a commercial production of electroplates on metals and is particularly concerned with a method or a process for predicting and eliminating the occurrence of pitting on the plate. For many years, little trouble was experienced in pitting during the electrodeposition of metal such as nickel on steel, copper and brass at low temperature and at low current density and high pH, for in the early period of commercial plating, a nickel surface that would buff to a nickel color was all that the trade required. Recently, however, particularly since nickel has been extensively used as a protective coating for automotive parts, it has become necessary to plate heavier deposits to withstand corrosion over longer periods of time. This has necessitated an increase in current densities and other operating conditions to facilitate the deposition of nickel in the least possible time. For some time, copper was thought to be necessary as a base on which nickel should be plated, but only recently, experience has shown that copper as an alternate plate between nickel and steel did not offer any protection for the base metal, but instead, contributed to the corrosion of either the steel or iron on account of its position in the electromotive series with respect to iron. Consequently, copper has been eliminated and nickel has been plated directly upon the steel. While pitting became readily apparent when the current densities were increased, it became a serious commercial problem as soon as the intermediate copper plate was discontinued.

We have made extensive researches into the origin of pits and we have established that there are many types and kinds of pits. For example, we have found that if an article is not properly cleaned or rinsed, it will retain small particles of foreign matter which will cause a steady stream of hydrogen which will interfere with the deposition, and that pitting results whenever such articles of dirt interfere with the uniform release of hydrogen.

We have also found that pitting is formed when a deep abrasion or scratch is present on the surface of the base metal, as such occurrence also interferes with the normal evolution of hydrogen during plating. Obviously, pitting which resulted from the foregoing conditions could be controlled upon proper treatment of the base metal, but even when diligent efforts were made to correct such conditions, pitting was found to result when all of the other known causes were eliminated.

Microscopic studies of the nickel structure even under the most favorable conditions of plating revealed startling facts. For example, it was found that nickel plated upon copper had a finer grained structure than that placed upon steel. Again, nickel plated at high temperature was coarser than that plated at low temperature and moreover nickel plated at high current densities was coarser than that plated at low current densities, but in every case, it was found that a finer grained, smoother surface would be substantially free from pits.

Commercial plating as heretofore practiced, has generally included the use of an addition agent, such as hydrogen peroxide, to the nickel bath for the alleged purpose of preventing pitting; and under such practices, the operator would replenish the tank at frequent intervals approximately such for example as every two hours, with a certain quantity of the addition agent which had previously been discovered by the trial and error method as being necessary to prevent pitting in any particular tank. The difficulty with such procedure, however, has been that the repeated replenishment has not prevented pitting; that it has been expensive and that it has required attention at too frequent intervals for assurance of safety.

It has been assumed that hydrogen peroxide would eliminate the pitting at any depth, but we have found that regardless of the amount used, satisfactory commercial plating on steel beyond a depth of six ten thousandths of an inch could not be effected, while satisfactory commercial plating on metals other than steel beyond a depth of one and one-fourth thousandths of an inch could not be obtained.

We have discovered that there is a definite relationship between pitting and grain size and that if the grain size is controlled, pitting can be eliminated. We have also discovered that even when hydrogen peroxide is used, the grain structure assumes the shape of an inverted cone with the apex end in contact with the base metal, and that such formation necessarily limits the depth of the plate, because as the depth increases, the base of the cone reaches a size that is beyond the limit of safe commercial plating. We have discovered that by the use of certain addition agents, the shape of the grain structure can be modified so as to form a column of uniform cross sectional shape throughout its length and that by reason of such formation, the depth to which the metal can be plated, can be safely increased in production to one and one-half times.

thousandths of an inch. In fact, we have been able to plate nickel on steel to a depth of forty-five thousandths of an inch and still maintain at the surface the grain size necessary to avoid pitting.

An object of our invention therefore, is to provide an indicator by means of which the conditions in a plating bath can be determined sufficiently far in advance to avoid loss by pitting.

10 In this connection, our invention is concerned with a method of plating by means of which, the pitting can be eliminated regardless of the depth of plate that is required for commercial production.

15 To illustrate the relationship between grain size and pitting, we have shown in Figs. 1 to 4, microphotographs which illustrate a gradual reduction in grain size of electrodeposited nickel; the grains being indicated at *a*, *b*, *c*, and *d* respectively. Fig. 5 is a cross sectional view on a greatly enlarged scale showing the grain structure of the nickel deposit on steel with the use of materials which have heretofore been known to the trade as addition agents to prevent pitting, while Fig. 6 is a similar cross sectional view showing the grain structure of a plate that is deposited in accordance with our invention.

It is well known that certain addition agents 30 produce advantageous results in electroplating, but the function of the agents has not been fully understood, and no general rule has been known that would enable one to predetermine the type of agent that would produce the most beneficial 35 results for a given set of conditions.

So far as we know, no one, heretofore, has ascertained that a definite relationship exists between grain size and pitting; moreover, although 40 addition agents have been used, they have not permitted nickel plating on steel to be accomplished at depths greater than six ten-thousandths of an inch. Furthermore, the addition agents have not eliminated the necessity for 45 constant supervision of bath conditions, and where hydrogen peroxide has been used, the cost has been an important factor in the operation of a plating plant.

Our invention is applicable for the plating of metals other than nickel, but by way of illustration, a satisfactory nickel bath is as follows:—

|                         | Oz. per gallon<br>of solution |
|-------------------------|-------------------------------|
| <chem>NiSO4.7H2O</chem> | 32                            |
| <chem>NiCl2.6H2O</chem> | 6                             |
| <chem>H3BO3</chem>      | 4                             |

The pH of this bath can be adjusted between 2 to 5.8 and electrolyzed with a current density of 5 to 400 amps. per sq. ft. at temperatures which 60 vary from room to boiling.

We have found that if the above-mentioned bath is used, for example, at room temperature and with a current density of 5 amps. per sq. ft., the resulting grain structure will be similar to that indicated in Fig. 4; but satisfactory commercial plating in large scale production cannot be accomplished at such low current density. In fact, it is necessary to use densities of approximately 75 amps. per sq. ft., and at such 70 densities, the grain structure would be changed to that illustrated in Fig. 1, under which conditions pitting would result.

To eliminate pitting and at the same time to maintain uniform grain size throughout the entire depth thereof, we have discovered that cer-

tain addition agents if added to the bath will not only eliminate pitting, but will also enable metal such as nickel, cadmium, cobalt, zinc and tin to be plated to depths which heretofore have been considered impractical for commercial work. 5 Such addition agents may comprise any one of the following:—

|                                                                                                                                                                     | Grams per gallon         |
|---------------------------------------------------------------------------------------------------------------------------------------------------------------------|--------------------------|
| Phenol                                                                                                                                                              | in the proportions of 2½ |
| Naphtha-quinone                                                                                                                                                     | do 1 10                  |
| Phenolphthalein                                                                                                                                                     | do 1½                    |
| The electrolyte soluble acid salts such as sulphides, chlorides, cyanides, carbonates and fluorides of metals, such as nickel, cadmium, zinc, tin, cobalt, and lead | do 2 15                  |
| The electrolyte soluble compounds, such as the hydroxides and oxides of metals, such as nickel, cadmium, zinc, tin, cobalt and lead                                 | do 2 20                  |

Where the term "salt" is used in the claims it is intended to include not only the addition of a salt per se, but also the addition of compounds which produce salts in the bath.

The phenol, naphtha-quinone and phenolphthalein may be grouped under a heading of chemicals which have a closed carbon chain.

In using the addition agents, we prefer to use the alkaline salts of the metals in alkaline plating baths, and we prefer to use the acid salts of the metals in neutral and acid plating baths. Furthermore, in using the metallic salts, we use a dissimilar metal for the addition agent from that metal which is to be plated in the bath. For example, in a nickel plating bath, we use any metallic salt mentioned other than that of nickel, and for cadmium, we use any metallic salt other than that of cadmium, etc.

The addition agents which we have mentioned have produced a very marked change in the grain formation. In Fig. 5, for example, 10, indicates a base metal such as steel, and 11 indicates a layer of nickel that has been affixed to the steel by electrodeposition. The lines 12 leading upwardly from the base metal to the outer surface of the plate represent the grain formation of the plated metal when an addition agent, such as hydrogen peroxide, is used in the bath. The grain formation is similar to an inverted truncated cone and accordingly it will be apparent that as the thickness of the plate increases, the size of the grain at the surface increases. As the grain size increases to about five thousandths of a millimeter, pitting develops, and consequently satisfactory commercial plating of nickel on 55 steel has not been accomplished in depths in excess of six ten thousandths of an inch; and so far as we know, pitting develops in the deposition of nickel at commercial rates on metals other than steel when the depth of plate exceeds one 60 and a quarter thousandths of an inch.

By the use of addition agents which we have mentioned, we have modified the formation of the grain to that illustrated in Fig. 6, in which the lines 15 represent the grain formation in the 65 plated metal. Such grains have uniform cross-sectional columnar shape throughout their length and hence there is no limit of depth to which the metal can be plated in satisfactory commercial production. So long as addition agents are 70 used in the proportions mentioned, the grain size will be approximately one thousandth of a millimeter and therefore entirely safe for commercial production.

To ascertain conditions in the bath, we exam- 75

ine a plated article, which is taken from the production line, either under a microscope and compare the grain size by observation with plates of known grain size, or we measure the image on the 5 ground glass plate of a microphotographic camera. So long as the grain size remains below five thousandths of a millimeter, no addition agents need be used, the bath being merely replenished with water so as to maintain the desired level. 10 If, however, we find that the grain size is increasing beyond the desired limit, then we add one of the hereinbefore addition agents in sufficient quantity to effect the desired grain size reduction. The total amount to be added will vary with the 15 size of the tank.

To illustrate the relationship between grain size and pitting, we have shown microphotographs in Figs. 1 and 2, in which the grain size is over eight thousandths of a millimeter; the 20 illustration in Fig. 1 being coarser than that of Fig. 2. In Fig. 3, the grain size is approximately five thousandths of a millimeter, while in Fig. 4, the grain size is approximately one thousandth of a millimeter. The article illustrated in Fig. 1 was found to be very badly pitted, while in Fig. 2 has a slight reduction in grain size with a 25 corresponding reduction in the number of pits. The article illustrated in Fig. 3 has a grain size in which very little pitting will occur, while that presented in Fig. 4 is well within the range of 30 commercial plating and free from pits.

We have found when the grain size of grey nickel is controlled between one thousandth and five thousandths of a millimeter, that the articles 35 will be accepted commercially as being free from pits. Gray nickel as referred to herein and as defined in the trade means a plate which has a non-lustrous or non-image producing surface and is distinguished from bright-plate which has a 40 lustrous or image-producing surface. Bright nickel plate has a grain size of approximately one ten-thousandth of a millimeter in which range pitting, due to grain size, does not occur.

Our invention possesses important commercial 45 advantages for it has entirely eliminated pitting and yet, has enabled metal to be plated on steel at depths heretofore considered impossible for commercial production. The invention is not limited to nickel plating, but is well adapted for 50 plating other materials such as cadmium, zinc and tin. In the case of cadmium plating, a suitable bath prior to the introduction of the addition agent is as follows:—

|                     | Oz. per gallon |
|---------------------|----------------|
| 55 NaCN             | 10             |
| Cd(CN) <sub>2</sub> | 4.5            |
| NaOH                | 7              |

In the case of zinc plating, a suitable bath prior 60 to the introduction of the addition agent is as follows:—

|                     | Oz. per gallon |
|---------------------|----------------|
| Zn(CN) <sub>2</sub> | 4              |
| NaCN                | 3.5            |
| NaOH                | 7              |
| 65 NaF              | 1/2            |

In the case of tin plating, a suitable bath prior 70 to the introduction of the addition agent is as follows:—

|                                         | Oz. per gallon |
|-----------------------------------------|----------------|
| 70 SnCl <sub>2</sub> .2H <sub>2</sub> O | 4              |
| NaOH                                    | 10             |

It is to be understood that the pH of these 75 various baths is adjusted, that they are electrolyzed at a current density similar to those used com-

mercially, and that an addition agent mentioned is to be added in the proportion specified.

We claim:—

1. A continuous homogeneous ductile electrolytic deposit of gray nickel directly on steel 5 wherein the deposit has a grain size between one-thousandth and five-thousandths of a millimeter and wherein the deposit exceeds six ten-thousandths of an inch in thickness and is free of pitting. 10

2. A continuous homogeneous ductile electrolytic deposit of gray nickel directly on steel wherein the deposit has a grain size between one-thousandth and five-thousandths of a millimeter and wherein the grains have a substantially columnar structure and wherein the deposit exceeds six ten-thousandths of an inch in thickness and is free of pitting. 15

3. A continuous homogeneous ductile electrolytic deposit of gray nickel on steel wherein the deposit has a grain size between one-thousandth and five-thousandths of a millimeter and wherein the deposit exceeds six ten-thousandths of an inch and is free of pitting, and wherein the deposit is maintained within the aforesaid grain 20 sized limits by the periodic determination of the grain size of the deposit and by adding to the bath an addition agent having the property of reducing the grain size of the deposit in a sufficient quantity to restrict the grain size of the deposit to a value below that at which pitting, due to grain size, occurs, but above that of bright nickel, when the grain size approximates the upper limit stated. 25

4. An electroplating bath for the electro-deposition of a continuous homogeneous ductile gray deposit of nickel, substantially consisting of a solution of nickel sulphate, nickel chloride and boric acid, and an addition agent selected from the group consisting of a soluble salt of cadmium, 30 zinc, tin, cobalt and lead in the quantity of substantially two grams per gallon. 35

5. A method of avoiding the occurrence of pitting in the electro-deposition of metals of the group consisting of nickel, zinc, cadmium, cobalt 45 and tin, under conditions which otherwise would normally produce a grain size growth at which pitting would occur, comprising maintaining in the bath an addition agent, having the property of reducing the grain size of the deposit, in a quantity sufficient only to produce a deposit, the grain size of which is below, but substantially of the order of that at which pitting, due to grain size, occurs. 50

6. A method of avoiding the occurrence of pitting in the electro-deposition of gray nickel, under conditions which otherwise would normally produce a grain size growth at which pitting would occur, comprising maintaining in the bath an addition agent, having the property of reducing the grain size of the deposit, in a sufficient quantity to restrict the grain size of the deposit to a value below that at which pitting, due to grain size occurs, but above that of bright nickel. 60

7. A method of avoiding the occurrence of pitting in the electro-deposition of gray nickel under conditions which otherwise would normally produce a grain size growth at which pitting would occur, comprising electrolyzing a bath at a current density in the neighborhood of 75 amperes per square foot of cathode surface or higher, maintaining in the bath an addition agent having the property of reducing the grain size of the deposit, in a sufficient quantity to restrict the grain size of the deposit to a value 70 75

below that at which pitting, due to grain size occurs, but above that of bright nickel.

8. A method of avoiding the occurrence of pitting in the electro-deposition of gray nickel under conditions which otherwise would normally produce a grain size growth at which pitting would occur, comprising maintaining in the bath an addition agent having the property of reducing the grain size of the deposit selected from a group consisting of a soluble salt of zinc, cadmium, cobalt, lead and tin in a sufficient quantity to restrict the grain size of the deposit to a value below that at which pitting, due to grain size occurs, but above that of bright nickel.
15. 9. A method of avoiding the occurrence of pitting in the electro-deposition of zinc under conditions which otherwise would normally produce a grain size growth at which pitting would occur, comprising maintaining in the bath an addition agent having the property of reducing the grain size of the deposit, said agent being an electrolyte soluble metal salt in a quantity sufficient only to produce a deposit, the grain size of which is below but substantially of the order of that at which pitting, due to grain size, occurs.

10. A method of avoiding the occurrence of pitting in the electro-deposition of tin under conditions which otherwise would normally produce a grain size growth at which pitting would occur, comprising maintaining in the bath an addition agent having the property of reducing the grain size of the deposit, said agent being an electrolyte soluble metal salt in a quantity sufficient only to produce a deposit, the grain size of which is below but substantially of the order of that at which pitting, due to grain size, occurs.

11. A method of avoiding the occurrence of pitting in the electro-deposition of gray nickel under conditions which otherwise would normally produce a grain size growth at which pitting would occur, comprising electrolyzing a bath at a cathode current density in the neighborhood of 75 amperes per square foot or over and maintaining in the bath an addition agent having the property of reducing the grain size of the deposit selected from the group consisting of a soluble salt of zinc, cadmium, cobalt, lead and tin in a sufficient quantity to restrict the grain size of the deposit to a value below that at which pitting, due to grain size, occurs but above that of bright nickel.

12. A method of avoiding the occurrence of pitting in the electro-deposition of gray nickel under conditions which otherwise would normally produce a grain size growth at which pitting would occur, comprising maintaining in a sulphate bath an addition agent having a property of reducing the grain size of the deposit, selected from a group consisting of a soluble salt of zinc, cadmium, cobalt, lead and tin in a sufficient quantity to restrict the grain size of the deposit to a value below that at which pitting, due to grain size, occurs, but above that of bright nickel.

13. A method of avoiding the occurrence of pitting in the electro-deposition of zinc under conditions which otherwise would normally produce a grain size growth at which pitting would occur, comprising maintaining, in a cyanide bath, an ad-

dition agent having the property of reducing the grain size of the deposit, said agent being an electrolyte soluble metal salt in a quantity sufficient only to produce a deposit, the grain size of which is below but substantially of the order of that at which pitting, due to grain size, occurs.

14. A method of avoiding the occurrence of pitting in the electro-deposition of tin under conditions which would otherwise normally produce a grain size growth at which pitting would occur, comprising maintaining in a stannate bath an addition agent having the property of reducing the grain size of the deposit, said agent being an electrolyte soluble metal salt in a quantity sufficient only to produce a deposit, the grain size of which is below but substantially of the order of that at which pitting, due to grain size, occurs.

15. A method of avoiding the occurrence of pitting in the electro-deposition of gray nickel under conditions which otherwise would normally produce a grain size growth at which pitting would occur, comprising electrolyzing a sulphate bath at a current density in the neighborhood of 75 amps. per square foot or over, and maintaining in the bath an addition agent having the property of reducing the grain size of the deposit selected from the group consisting of a soluble salt of zinc, cadmium, cobalt, lead and tin in a sufficient quantity to restrict the grain size of the deposit to a value below that at which pitting, due to grain size occurs, but above that of bright nickel.

16. A method of avoiding the occurrence of pitting in the electro-deposition of gray nickel under conditions which otherwise would normally produce a grain size growth at which pitting would occur, comprising maintaining in a sulphate bath which is adjusted to a pH of from 2 to 5.8 an addition agent having the property of reducing the grain size of the deposit and selected from a group consisting of a soluble salt of zinc, cadmium, cobalt, lead and tin in a sufficient quantity to restrict the grain size of the deposit to a value below that at which pitting, due to grain size occurs, but above that of bright nickel.

17. A method of avoiding the occurrence of pitting in the electro-deposition of gray nickel under conditions which otherwise would normally produce a grain size growth at which pitting would occur, comprising maintaining in the bath an addition agent having the property of reducing the grain size of the deposit and selected from a group consisting of a soluble salt of zinc, cadmium, cobalt, lead and tin and in a quantity of substantially two grams per gallon.

18. A method of avoiding the occurrence of pitting in the electro-deposition of gray nickel under conditions which otherwise would normally produce a grain size growth at which pitting would occur, comprising maintaining in the bath an addition agent having the property of reducing the grain size of the deposit, said agent being an electrolyte soluble metal salt in a quantity sufficient to restrict the grain size of the deposit to a value below that at which pitting, due to grain size, occurs, but above that of bright nickel.

CERTIFICATE OF CORRECTION.

Patent No. 2,119,304.

May 31, 1938.

EUGENE D. VIERS, ET AL.

It is hereby certified that the above numbered patent was erroneously issued to "Eaton Detroit Metal Company" whereas said patent should have been issued to Eaton Manufacturing Company, of Cleveland, Ohio, a corporation of Ohio, as assignee by mesne assignments, as shown by the record of assignments in this office; and that the said Letters Patent should be read with this correction therein that the same may conform to the record of the case in the Patent Office.

Signed and sealed this 9th day of August, A. D. 1938.

Leslie Frazer

(Seal)

Acting Commissioner of Patents.